

# United States Patent Office

3,169,863

Patented Feb. 16, 1965

1

3,169,863

## PENTAERYTHRITOL PHOSPHORIC ACID ESTER SENSITIZERS FOR PHOTOGRAPHIC EMULSIONS

Herbert Grähöfer, Cologne-Flittard, Herbert Müller, Leverkusen, Rolf-Fred Posse, Cologne-Flittard, and Hans Ulrich, Leverkusen, Germany, assignors to Agfa Aktiengesellschaft, Leverkusen, Germany, a corporation of Germany

No Drawing. Filed June 11, 1963, Ser. No. 286,924  
Claims priority, application Germany, July 21, 1962,

A 40,784

9 Claims. (Cl. 96—66)

The invention relates to chemical sensitizers for photographic emulsions, to photographic emulsions and developer compositions containing these and to the production of photographic images in the presence of said sensitizers.

In the graphic arts field, particularly for raster photography, more and more films are being used which are on the market as so-called lithographic or line films and which can be developed to very high gamma values and therefore sharp raster points in developers which contain formaldehyde.

Although the processing of such films in developers containing formaldehyde gives excellent results, it must be carried out with great care. The interval during development in which a sharp raster point is obtained, i.e. the steepest gamma, is only short. It amounts to approximately between  $\frac{1}{2}$  and  $1\frac{1}{2}$  minutes.

It is known to add phosphorylated alkylene oxide derivatives to photographic silver halide emulsions to improve the mechanical properties thereof. However, these compounds are unsuitable for obtaining a high contrast.

It has now been found that the gamma values of photographic emulsions and the period during development in which an extremely high gamma value is obtained can be increased, so that development can be carried out much more effectively and conveniently, if the development is carried out in the presence of spirocyclic phosphoric acid esters which are obtainable by reaction of spirocyclic pentaerythritol-di-(phosphoric acid monohalides), particularly -(monochlorides) of the formula



with polyglycols of the formula



These spirocyclic pentaerythritol-di-(phosphoric acid monohalides) are also known as pentaerythritol esters of phosphorochloridic acid.

The degree of polymerization  $n$  of the glycol may be 3 or more, for instance 3-100, preferably 4-50. To prepare the esters, the glycols specified are preferably used in quantities of about 1 to 2 mole per mole of the halides.

The products obtained from the reaction of the above components are generally water-soluble and presumably have the following constitution:



In this formula,  $n$  has the meaning given above, and the degree of condensation  $X$  of the product of esterification may be 1 or more, for instance 1-100, preferably 1-10. In the above hypothetical formula, the substituent  $R$  may represent H or



2

The effect of these compounds in the development of lithographic films was all the more surprising in view of the fact that short chained polyethylene glycols as well as octaethylene glycol are ineffective, and comparable spirocyclic compounds with carbon as the ring atom, e.g. compounds of the following formula where  $n$  and  $X$  have the meaning given above:



do not produce extremely high gamma values.

Any silver halide emulsions of the developing-out type which provide a high gamma when developed with developers containing formaldehyde may be used. The silver salts of such emulsions generally consist of silver chloride in a quantity of at least 50 mole percent. However, it is preferred to use emulsions in which the silver salts consist at least of 65 mole percent of silver chloride and accordingly 35 mole percent or less of silver bromide. The emulsions may further contain small amounts of silver iodide, such as 1 to 2 mole percent.

The quantity of the above phosphoric acid esters to be added to the emulsion depends on the ratio of chloride to bromide in the emulsion, 10 to 100 mg. per mol of silver halide may advantageously be used. The emulsions can in addition be chemically sensitized with salts of noble metals, such as gold salts, with sulfur compounds or with reducing agents. Moreover the emulsions can be optically sensitized with cyanine and merocyanine dyes.

The developers which may be employed in our invention contain as essential components a phenol type developer, such as hydroquinone, an alkali, such as an alkali metal carbonate, sodium or potassium carbonate, formaldehyde bisulfite and a small amount of a restrainer, such as alkali metal bromide. If desired the developer can also contain sodium hydroxide, boric acid, a sequestering agent. Instead of alkali metal carbonate and formaldehyde bisulfite the developer can contain, as a source of formaldehyde, paraformaldehyde, an alkali metal sulfite and a buffering agent, such as alkali metal bisulfite. Such developers are well known in the art and are for instance disclosed in U.S. Patents 2,184,053, 2,313,523, 2,902,367 and in British Patent 643,411. Such developers may contain for instance per one liter 15-25 grams of hydroquinone, 30-70 grams of formaldehyde bisulfite, 30-90 grams of sodium carbonate monohydrate, 5-20 grams of boric acid and 1-5 grams of alkali metal bromide or 15-25 grams of hydroquinone, 5-10 grams of paraformaldehyde, 1-5 grams of potassium metabisulfite (cryst.), 20-40 grams of anhydrous sodium sulphite, 5-15 grams of boric acid and 1-5 grams of alkali metal bromide.

The phosphoric acid esters of the present invention may be added to the above lithographic developers preferably in quantities of 30-300 mg. per liter.

The addition of the phosphoric acid esters of the present invention to the emulsion and/or to the developer causes the gamma value to rise considerably during development, for instance from about 6-8 to above 15. At the same time, the margin of time during development within which sharpness of raster dots may be obtained is increased from about one minute to 3 to 4 minutes. Furthermore, a formaldehyde containing developer having such an addition is less dependent upon temperature. Whereas a developer without this addition reacts to temperature increases of 1 to 2°C. with a marked reduction in the margin of time for development, good results may be obtained with developer temperatures of 15 to 40°C. if these phosphoric acid esters have been added. Owing to the increased time available for processing, the above



used as casting additives, are added to the emulsion per mole of silver halide:

- (B) +80 mg. octaethylene glycol
  - (C) +80 mg. Compound VII
  - (D) +80 mg. Compound I

All the samples are illuminated in a sensitometer behind a grey step wedge and developed for 5 minutes at 18° C. in a developer of the following composition:

|                                | G.   |
|--------------------------------|------|
| Anhydrous sodium sulphite      | 30   |
| Boric acid                     | 7.5  |
| Hydroquinone                   | 22.5 |
| Potassium metabisulphite       | 2.5  |
| Paraformaldehyde               | 7.5  |
| Potassium bromide              | 1.5  |
| Diluted to 1 liter with water. |      |

## Result:

|              | Gamma | Fog  | 20 |
|--------------|-------|------|----|
| Experiment A | 6     | 0.04 |    |
| Experiment B | 6     | 0.04 |    |
| Experiment C | 6     | 0.04 |    |
| Experiment D | 15    | 0.04 |    |

### Example 2

An emulsion according to Example 1 is divided into two portions. One portion (A) has no additive while the other portion (B) has added to it 80 mg. of Compound II per mole of silver halide. Each portion is then poured on to a film base. The two samples are then illuminated and developed as in Example 1.

## Result:

|            | Gamma | Fog  |
|------------|-------|------|
| Emulsion A | 7     | 0.05 |
| Emulsion B | >15   | 0.05 |

### Example 3

An emulsion according to Example 1 is divided into a portion (A) without additive and a portion (B) with 80 mg. of Compound III per mole of silver halide as additive, and the portions are poured on to a base and then treated as described under 1.

## Result:

|                 | Gamma | Fog  |
|-----------------|-------|------|
| Emulsion A----- | 6     | 0.04 |
| Emulsion B----- | >15   | 0.04 |

*Example 4*

Film strips (Agfa-lith-ortho) illuminated behind a stepped wedge are developed in the developer mentioned in Example 1 for varying time ranging from 1 to 4 minutes, at 20° C. The same film samples are developed in the same developer after the addition of 100 mg./liter of Compound I.

## Results

|                             | 1'  | 1½' | 2'  | 2½' | 3'  | 4' |
|-----------------------------|-----|-----|-----|-----|-----|----|
| Gamma without additive----- | 7.5 | 15  | 12  | 6.5 | 5.5 | 5  |
| +100 mg. I/l-----           | 10  | >15 | >15 | >15 | >15 | 15 |

What we claim is:

1. In a process for the production of photographic images by developing silver halide emulsion layers in which the silver halide has a silver chloride content of at least 50 mole percent with photographic developer solutions containing formaldehyde, the improvement which comprises carrying out said development in the presence of a condensation product of a pentaerythritol ester of phosphorochloridic acid and a polyethylene glycol with a degree of polymerization of at least 3.
  2. A process as defined in claim 1 in which the condensation product is the condensation product of one mol of a pentaerythritol ester of phosphorochloridic acid and about 1 to 2 mols of a polyethylene glycol.
  3. A process as defined in claim 1 in which the condensation product has the formula



wherein R represents a member of the group consisting of hydrogen and radicals having the formula



in which  $n$  represents an integer of at least 3 and  $X$  represents an integer of at least 1.

- 30 4. A light-sensitive photographic material comprising a silver halide emulsion layer in which the silver halide has a silver chloride content of at least 50-mol percent, which contains a condensation product as defined in  
35 claim 1.

5. A light-sensitive photographic material comprising a silver halide emulsion layer in which the silver halide has a silver chloride content of at least 50-mol percent, which contains a condensation product as defined in  
40 claim 2.

6. A light-sensitive photographic material comprising a silver halide emulsion layer in which the silver halide has a silver chloride content of at least 50-mol percent,  
45 which contains a condensation product as defined in claim 3.

7. Photographic developing composition comprising hydroquinone and formaldehyde, which contains in addition a condensation product as defined in claim 1.

50 8. Photographic developing composition comprising hydroquinone and formaldehyde, which contains in addition a condensation product as defined in claim 2.

9. Photographic developing composition comprising hydroquinone and formaldehyde, which contains in addition a condensation product as defined in claim 3.

**References Cited in the file of this patent**

UNITED STATES PATENTS

|           |                |       |               |
|-----------|----------------|-------|---------------|
| 2,531,832 | Stanton        | ----- | Nov. 28, 1950 |
| 2,956,881 | Van Lare       | ----- | Oct. 18, 1960 |
| 2,961,317 | Webster et al. | ----- | Nov. 22, 1960 |
| 2,974,158 | Lanham         | ----- | Mar. 7, 1961  |
| 3,005,007 | Fierce et al.  | ----- | Oct. 17, 1961 |
| 3,090,799 | Wahl et al.    | ----- | May 21, 1963  |